

# UNITED STATES PATENT OFFICE.

HENRY DREYFUS, OF LONDON, ENGLAND.

## MANUFACTURE OF COMPOSITIONS, PREPARATIONS, OR ARTICLES HAVING A BASIS OF CELLULOSE ACETATE.

1,353,384.

Specification of Letters Patent. Patented Sept. 21, 1920.

No Drawing.

Application filed April 15, 1919. Serial No. 290,316.

To all whom it may concern:

Be it known that I, HENRY DREYFUS, a citizen of the Swiss Republic, residing at London, England, have invented certain 5 new and useful Improvements in or Relating to the Manufacture of Compositions, Preparations, or Articles Having a Basis of Cellulose Acetate, of which the following is a specification.

10 In the manufacture of non-inflammable celluloid with cellulose acetate it is essential to have solvents of high boiling point, especially solvents which have a higher boiling point than 300° C. Moreover it is necessary 15 for general use of the products that such bodies shall really be solvents at a low temperature, at least at ordinary temperature, or even at 0° C. or it may even be far below, especially if the non-inflammable celluloid is used for articles such as aeroplanes or airships, which are exposed to very low temperatures. It follows that the bodies referred to must not be merely liquids such as castor oil, for instance, which have no solvent power for cellulose acetate at low temperature and only serve to make the material softer; on the contrary the body must be a real solvent, which dissolves the cellulose acetate at a low temperature, or even at a very low temperature, to a clear solution, even when the solution is in a concentrated form, and which solution remains clear if it is cooled down to a low temperature.

If one merely takes a softening oil which has no solvent action on the cellulose acetate, this takes away the strength of the manufactured articles, such for instance as celluloid masses, sheet, films or articles manufactured in any form, because the more the quantity of such non-solvent softening oil is increased the greater is the reduction in the strength of the celluloid or articles so made. If however one has a real solvent, which at the same time is not a solid body at ordinary or low temperature, the strength of the product always remains the same, even if one adds more of this softening agent or solvent in or to the non-inflammable celluloid to obtain desired degrees of softness or pliability. In other words the articles made may be hard and stiff, or soft, or they may be so soft that they are pliable like an ordinary fabric.

Such solvent of high boiling point, besides being liquid or not a solid body at or-

dinary or low temperature, should also be insoluble in water, especially boiling water, so as to render all the non-inflammable celluloid made with it water-proof in any condition, whether the celluloid is very thick 60 and at the same time hard, or whether it is in the form of very thin sheets and hard (in which case it is much more easily attacked by water or humidity), or whether it is made so soft that it becomes pliable like fabric (in this case if it is very thin and not waterproof it is not resistant at all). Furthermore such a solvent must be neutral, not acid nor alkaline nor liable to become so by boiling with water.

The before-mentioned conditions therefore imply also that such solvent cannot be a substance having a melting point of say 40° or 50° C. for example, or even less. It must be a liquid or not a solid material at ordinary temperature, and preferably at zero or even below zero, for instance in some cases even as low as minus 18° C., this being more particularly important for applications such as airships and aeroplanes.

If it has the qualities above mentioned, besides non-inflammability, then from every point of view it can be used for any application in the manufacture of non-inflammable celluloid, whether it be for very thin sheets such as films, for windows, or for making celluloid sheets in any form, pliable like fabrics or for thick plates or blocks, or for any other applications for which cellulose acetate can be used.

The plastic-inducing solvents fulfilling these conditions have not been known up to the present day.

It was proposed long ago that one should use triphenylphosphate as a solvent for 95 cellulose acetate. Triphenylphosphate is a product having a high boiling point (over 300° C.) but it has a melting point of 40° to 50° C., and even at this melting point is not a solvent of any cellulose acetate at ordinary temperature, although it has been proposed and considered as a solvent in different quarters; it only acts as a solvent at and above 150° C., and ceases to be a solvent at a temperature a little lower than 150° C., at ordinary temperature it does not dissolve at all, any acetate of cellulose. The only property which it has is to render the material less inflammable or non-inflammable; it decreases the combustibility, and this in 110

such a way that according to the increase of the quantity of triphenylphosphate relatively to the quantity of cellulose acetate employed, one has a sliding scale up to in- 5 combustibility, and it may be assumed that with about 10% to 15% of triphenylphosphate one gets a maximum incombustibility of the so-formed celluloid of any form and size.

10 As triphenylphosphate is not a solvent for cellulose acetate at ordinary temperature it decreases the strength of the articles made therewith. If the quantity above mentioned is increased on the supposition that it is a 15 solvent, then one would have the negative effect, inasmuch as the celluloid so formed would become cloudy and more and more lacking in strength, because in increasing this quantity of triphenylphosphate one 20 weakens the consistency and coherence of the celluloid, as the celluloid is permeated by a product which is not a solvent. This besides the fact that it would not be an appropriate solvent (even if it were a solvent) 25 owing to its being a solid.

The use of triphenylphosphate in connection with nitro-cellulose was first proposed in American Patent No. 733110, and the use 30 of this material in connection with cellulose acetate was proposed in the American Patent No. 729990 where it is also explained how the material was used in connection with cellulose acetate without result, owing to the brittleness of the resulting products.

35 Later, in other publications, its use has from time to time been suggested, but always considering it as a solvent, in spite of the fact that it is not a solvent, and its use is always for the same purpose as explained in the aforesaid American patents.

The same thing applies to tricresylphosphate. Tricresylphosphate has also a high 45 boiling point, and it has an advantage over triphenylphosphate in that it is liquid at ordinary temperature and even at a low temperature, but though liquid, it has no solvent power for acetate of cellulose at ordinary temperature. It acts similarly to castor oil; although it is much better than 50 castor oil, inasmuch as at higher temperatures it is a real solvent, whereas castor oil is not and is actually repellent to cellulose acetate. At the same time, however, tricresylphosphate has the effect of rendering 55 the product more incombustible, according to the quantity used, in the same way as triphenylphosphate. In any case a satisfactory celluloid could not be made with it alone because if the cellulose acetate was 60 used with it alone, the product could not be transformed into a plastic mass which could be afterward converted by the usual processes into celluloid of any form, for example in using at the same time, as usual, liquids 65 of low boiling point such as acetone, methyl

acetate and so forth. If it were then attempted to make a celluloid mass in the usual kneading apparatus, a mass would result which would seem to be a plastic mass; but, as soon as this was brought on to rollers 70 and the low boiling liquids allowed to evaporate, the mass would become dry and lose its consistency and coherence, because all the solvents would evaporate and the mass become cloudy, brittle and of no use. 75 Uninflammable celluloid sheets could not even be formed, as they would all break.

It has also been suggested to use substances such as paratoluenesulfonamid, benzene sulfonamid and paraethyltoluenesulfonamid. These substances do not fulfil the requirements stated above, as they are not solvents at ordinary temperature and are moreover even solid at a relatively higher temperature, so that one is obliged to use 85 solvents in order to mix them together with cellulose acetate. If one heats to above the melting point of the substance and then introduces some cellulose acetate, this dissolves; but, as soon as the temperature goes 90 down, the substance crystallizes again and the cellulose acetate comes out of solution, and the solvent, being a solid body, crystallizes throughout the cellulose acetate. Thus, for example, paratoluenesulfonamid, the use 95 of which has been suggested several times, has a melting point much higher than 100° C. so that its use is out of the question.

I have now found that the necessary properties for the purposes referred to are possessed by mixtures of isomeric xlenemono-methylsulfonamids, mixtures of isomeric xlenedimethylsulfonamids and mixtures of isomeric xlenemonoethylsulfonamids, made 100 from crude or commercial xylene. 105

These substances represent mixtures of the isomeric alkylated amids (of o, m and p-xylene sulfonic acids) such as can be obtained by treating an ordinary commercial xylene, distilling for example at about 135° 110 to 146° C., and containing, as is known o, m and p-xlenes), by the ordinary methods of conversion into the alkyl sulfonamids, for example by treating the crude xylene with chlorosulfonic acid to form the corresponding sulfochlorids, and then with ammonia to convert these into the sulfonamids and then methylating same to the mono or dimethyl stage or ethylating to the mono-ethyl stage; or by treating the said mixed sulfochlorids with amines such as methylamin, ethylamin, etc. Such mixtures of isomeric xylene mono or dimethylated or monoethylated sulfonamids are hereinafter in the claiming clauses referred to as high boiling 120 mixtures, liquid at ordinary temperature, of isomeric xylene low-carbon-alkyl sulfonamids. 125

It is to be observed that the known substances, pure monomethylamid and pure di- 130

methylamid of 1,3 dimethylbenzene sulfonic acid, have melting points respectively of 43° C., and 35° C., and are unsuitable for the purposes of the invention. The above 5 mentioned mixtures containing the mixed isomerids referred to, however, are suitable. Naturally any mixtures of them may be employed or mixtures of them with other plastic inducing bodies, and the claims are to 10 be read accordingly.

The said substances are on the one hand very viscous liquids at ordinary temperature, even more viscous than castor oil, and on the other hand they have very high boiling 15 points, much higher than 300° C.; also they are good solvents for acetate of cellulose at ordinary temperature and even at zero or below zero C.; they are good solvents for acetate of cellulose, and they give 20 a clear solution, liquid or stiff according to the temperature and the relative quantities employed of the solvent and acetate of cellulose.

These solvents or plastic including substances, which have not previously been employed together with acetate of cellulose, have the property that at ordinary temperature they are liquid, and are not solid bodies 25 at zero C. or even at minus 10° C. or lower. 30 They become more viscous when cooled down and do not crystallize, which is an important feature in this invention.

Moreover, they have the property of being insoluble or practically insoluble in water, even in boiling water.

The said solvents are therefore eminently suitable for use for the manufacture of non-inflammable celluloid for any purpose, whether it be for making a very hard celluloid 40 or a less hard celluloid, or a very soft one, for thick sheets, or thin sheets or sheets which are pliable like fabric, or the stages between hard and pliable like a fabric. The products made with said solvents are water-resisting in a very high degree.

These solvents can also, in order to render them quite incombustible, be used together with triphenylphosphate, or preferably with tricresylphosphate or they may be used in 50 mixture with any other known camphor substitute for cellulose acetate.

In order to illustrate by way of example how the invention may be carried out in practice, one may use to 100 kilos of cellulose acetate, having for example a high viscosity, 25 kilos of the xylene monomethylsulfonamid solvent and 12 kilos of tricresylphosphate or triphenylphosphate, these substances being mixed together with solvents 55 of low boiling point, such as acetone or methyl acetate or ethyl acetate mixed with alcohol (four volumes to one volume of alcohol), the mass being worked in the ordinary way in the celluloid apparatus, first 60 in the mixers, then on the rollers and after-

ward in the presses and so on, as generally practised in the celluloid industry. This process gives quite a hard incombustible celluloid which can even be used at a low temperature without becoming brittle.

The quantity of 25 kilos of the xylene monomethylsulfonamid solvent may be reduced together with that of the triphenylphosphate or tricresylphosphate in order to get the celluloid still harder if required.

On the other hand by increasing the quantity of the xylene monomethylsulfonamid solvent one gets softer non-inflammable celluloid in proportion as the quantity is increased, until at last a celluloid is obtained 80 which is pliable like a fabric.

Of course the contents of my British specification No. 114304 (3336 of 1918) have to be taken into consideration in this connection, which specification indicates the relationship between the quantity of high boiling solvents used and the viscosity of the cellulose acetate, in the sense that the higher the viscosity of the cellulose acetate 85 the more of the solvent or plastic-inducing substance is to be used, and the less the viscosity of the cellulose acetate the less of the softening or plastic-inducing substance is to be used.

For example if one takes to 100 kilos of cellulose acetate, 100 kilos of the xylene monomethylsulfonamid solvent then one gets the kind of celluloid which is pliable like a fabric, and if one employs this solvent plastic-inducing substance in quantities less 90 than 100 per cent. calculated on the weight of cellulose acetate, one gets a proportionately stiffer celluloid, according to the reduction of the quantity of the solvent plastic-inducing substance, while if the quantity of the solvent plastic-inducing substance 100 is increased above 100 per cent. calculated on the weight of the cellulose acetate, a still more pliable celluloid is obtained.

In the various examples given above, the aforesaid xylene monoethyl sulfonamid solvent or the said xylene dimethyl sulfonamid solvent may be employed wholly or partly instead of the xylene monomethyl sulfonamid solvent.

The celluloids, non-inflammable films, articles or products having a basis of cellulose acetate obtained as above described are of especial value for aeroplane and airship purposes, as they retain the same properties 110 under the extreme conditions of heat and cold to which they are liable to be exposed in service and independent of conditions promoting evaporation and notwithstanding exposure to wind of any direction or velocity favoring evaporation. Besides the manufacture of celluloid the solvents of high boiling point of the present invention are 120 also very important for other manufactures 125 in which cellulose acetate is used in any 130

form and application—for example, for artificial silk, dope, films and other compositions of matter.

In the dope manufacture they are especially important inasmuch as if they are used as solvent plastic-inducing substance in the dope there remains after evaporation of the dope, a solid film mass which presents the greatest surface to the air, does not lose the plastic-inducing substance by evaporation and resists water, whereas if one only had a plastic-inducing substance of lower boiling point it would evaporate very quickly, so that the qualities of the dope imparted by such plastic-inducing substance would rapidly disappear, a specially serious drawback for dope for airships, while if the plastic-inducing substance used were not insoluble in water the dope would soon be washed away, thus quickly deteriorating the surface, such as balloon fabrics, and if the plastic-inducing substance used became solid at low temperatures it would lose its solvent power and then the surface of the film remaining on the surface would become brittle and consequently not resistant to water, a matter which is also important in connection with airships.

If, however, the solvent plastic-inducing substances of the present invention are used, all these difficulties can be avoided and one can make any quality required.

This is particularly essential for airships and aeroplanes, where the effects of low temperature and also the rapid evaporative effects caused by the high speed of the aeroplane or airship with or against the wind have to be taken into consideration both for the dope and for parts such as unbreakable windows and so forth.

Further, it has been known for a long time in the manufacture of celluloid to use urea in order to neutralize any trace of acid which may be developed, and urea is employed for the same purpose for cellulose acetate.

I have found that it is better to use, instead of urea, which has a high melting point, and therefore does not possess the same solvent capacity for cellulose acetate, urea derivatives of the aliphatic series which are either liquid or have a low melting point, such as monomethylurea, dimethylurea, trimethylurea, monoethylurea, diethylurea and so forth. They may be employed in about the quantities usual for urea.

Of course any other usual or suitable substances may be added to the solutions, mixtures or masses of the present invention or in making the same.

What I claim and desire to secure by Letters Patent is:

1. A composition of matter containing cellulose acetate, and containing a high-boiling mixture of isomeric xylene low-carbon-alkyl sulfonamids which mixture is liquid at ordinary temperature.

2. A composition of matter containing cellulose acetate, and containing a high-boiling mixture of isomeric xylene mono low-carbon alkyl sulfonamids which mixture is liquid at ordinary temperature.

3. A composition of matter containing cellulose acetate, and containing a high-boiling mixture of isomeric xylene monomethyl sulfonamids which mixture is liquid at ordinary temperature.

In testimony whereof I have hereunto subscribed my name.

HENRY DREYFUS.